

J. C. WOODRUFF,  
PROCESS OF ACTIVATING CARBON,  
APPLICATION FILED MAY 8, 1919.

1,368,987.

Patented Feb. 15, 1921.



Inventor  
John C. Woodruff  
by  
Francis D. Hardcastle

Attorney

# UNITED STATES PATENT OFFICE.

JOHN C. WOODRUFF, OF NEW YORK, N. Y.

## PROCESS OF ACTIVATING CARBON.

1,368,987.

Specification of Letters Patent. Patented Feb. 15, 1921.

Application filed May 8, 1919. Serial No. 295,624.

To all whom it may concern:

Be it known that I, JOHN C. WOODRUFF, a citizen of the United States, and residing at New York city, N. Y., have invented certain new and useful Improvements in Processes of Activating Carbon, of which the following is a specification.

This invention relates to the manufacture of absorbent carbon and has special reference to a process of rendering carbon, such as charcoal, highly active as an absorbent.

Heretofore, charcoal has been activated by means of steam in vertical tube furnaces called Dorsite treaters. This type of furnace consists of a nichrome tube symmetrically set in a vertical position and surrounded by a cylindrical combustion chamber heated to about 1100° C. by gas burners. On the inside of the above mentioned nichrome tube, there is concentrically located a nichrome steam pipe having part of its length perforated, and covered with nichrome wire cloth of rather fine mesh which is smaller than the particles of the material treated. The gaseous products of the reaction are drawn off through exhaust ports by means of a vacuum pump. Granular charcoal is introduced through a hopper valve feeding device at the top. The space surrounding the steam jet is kept full of carbon and as a portion is discharged from the bottom of the tube, thus lowering the level of the material in the tube, the level is replenished through the feed valve at the top of the furnace. Thus, a continuous gravity passage of the charcoal through the tube is maintained, unless interfered with by gas pockets, and the charcoal is activated by the superheated steam admitted through the steam jet.

The highest quality of absorbent charcoal is obtained only by running the material at a very slow rate or by re-running it several times through this type of furnace. This process requires a large amount of time and fuel. Difficulty is experienced in feeding due to the formation of gas pockets which hold the charcoal from sliding after the material is discharged from the bottom. The exhaust lines constantly give trouble by becoming plugged with charcoal.

One of the objects of this invention is to provide a process which is more efficient and simpler to operate than the prior processes; also cheaper and which may be conducted in a continuous manner and which will over-

come the disadvantages hereinbefore described in the prior processes.

Another object of this invention is to avoid the use of expensive nichrome tubes, 60 which usually burn out and also have the troublesome steam jets.

Reference is to be had to the accompanying drawings in which Figure 1 is a view in elevation of the apparatus used in my process, part of the device, however, being shown in section.

Fig. 2 is a section along the line 2—2 of Fig. 1.

This apparatus is similar to a cement kiln 70 in construction and operation and consists of a long slightly inclined cylinder (1), preferably of steel, and lined with a refractory substance (2), such as fire brick, and is mounted on rollers (3) so that it may be 75 rotated. The high end of the cylinder has a charging device (4) and an operating outlet (5) for the flue gases. At the lower end is a discharging device, shown in a diagrammatic way, by the pipe (6). A fire brick 80 box (7) at this end provides for the burning of coal, coke, powdered coal or tar-oil and is so built that the hot flue gases pass through the revolving tube. Steam, air, CO<sub>2</sub> or other oxidizing agents are also admitted 85 at this end.

Carbon is charged into the cylinder through the charging device (4) and as it passes through the cylinder it comes into contact with the hot flue gases and steam 90 at a high temperature, and the material becomes readily activated. It has been found that a temperature of 700° to 1100° C. produces satisfactory results.

With this internally fired rotary furnace, 95 a high percentage of yield may be obtained and the material may be produced in very large quantities. The peculiar efficiency of the process depends primarily upon the combined features of continuous agitation of 100 the carbon while undergoing oxidation and the delivery of the oxidizing and heating gases directly to the reaction chamber wherein they are mingled freely with the carbon while the required temperature is 105 readily maintained. By employing the heating gases directly, the heat is conserved and the process rendered rapid and economical. The uniform and highly active product may be used for a variety of purposes to 110 which it is adapted.

The furnace described is more economical

than the Dorsite apparatus from the standpoint of both installation and operation, and there are no expensive nichrome tubes to be burned out nor troublesome jets with which 5 to contend.

The present invention is not limited to the specific details set forth in the foregoing examples which should be construed as illustrative and not by way of limitation, and 10 in view of the numerous modifications which may be effected therein without departing from the spirit and scope of this invention, it is desired that only such limitations be imposed as are indicated in the appended 15 claims.

I claim as my invention:

1. A process of treating carbon by oxidation, which comprises, continuously agitating

ing the carbon while conveying it through a reaction zone and subjecting the carbon 20 while in said zone to the combined action of steam and hot combustion gases, the latter gases furnishing the necessary heat to maintain the temperature at a point insuring rapid activation of the carbon. 25

2. A process of treating carbon by oxidation, which comprises, continuously agitating the carbon while conveying it through a reaction zone and subjecting the carbon 30 while in said zone to the combined action of steam and hot combustion gases, the latter gases furnishing the necessary heat to maintain a temperature of between 700° C. and 1100° C.

JOHN C. WOODRUFF.